

Patented Feb. 13, 1951

2,541,822

# UNITED STATES PATENT OFFICE

2,541,822

## DI-(N-METHANE SULFONATES) OF DIARYL-ALKYLENE-DIAMINES AND THEIR USE FOR INHIBITING ACID-FADING

Donovan Erb Kvalnes, Penns Grove, N. J., and Carlton Webster Croco, Swarthmore, Pa., assignors to E. I. du Pont de Nemours & Company, Wilmington, Del., a corporation of Delaware

No Drawing. Application February 24, 1950,  
Serial No. 146,158

4 Claims. (Cl. 8—61)

1

This invention relates to novel organic compounds. More particularly this invention deals with water-soluble di-(N-methane sulfonates) of diaryl-alkylene-diamines.

It is an object of this invention to produce novel organic compounds useful as treating agents for textile fiber. A more specific object of this invention is to provide new agents for treatment of cellulose ester fiber in conjunction with the dyeing thereof, to render the dyeing stable against acid fume-fading. Additional, important objects of this invention will appear as the description proceeds.

It is known that materials consisting of or containing dyed cellulose acetate fibers tend to fade when they are exposed to an atmosphere containing oxides of nitrogen and sulfur. This is often referred to as acid- or gas-fume fading. This tendency is more troublesome because those parts of the cellulose acetate which are more directly exposed to fumes, e. g., the edges of a roll of cellulose acetate fabric, are more discolored than the interior areas. It so happens that storage houses wherein textile fabrics are stored in the course of commercial jobbing and distribution are commonly warmed in the winter by means of illuminating gas. The combustion products of the latter feed into the atmosphere oxides of nitrogen and sulfur, and thus produce exactly those conditions which are injurious to dyed cellulose acetate. The problem of gas-fume fading is thus one of great commercial significance.

It has been proposed in the art to treat cellulose ester fiber with special agents which will retard or inhibit the mentioned fading. Two types of materials have been suggested or actually used for this purpose:

1. *Water-soluble agents.*—These may be applied readily from aqueous solution after dyeing. They suffer, however, from the drawback of being readily washed out of the fiber. For this reason it is not practical to apply them to the fabric prior to dyeing or during the dyeing operation, inasmuch as the latter is generally followed by a soaping and rinsing step, which would obviously remove the inhibitor.

Furthermore, when the fabric is made into clothes the latter will upon laundering lose the inhibitor and become susceptible to gas-fume fading.

In addition, the customary water-soluble agents have the peculiar property of reducing the light fastness of viscose fiber when dyed with direct colors. Consequently, the inhibitors cannot be

2

applied to a combination fabric made up of cellulose ester and viscose fibers.

2. *Water-insoluble agents.*—These must be applied either from organic solvent solution or in the form of an aqueous suspension. Both of these methods, however, are burdensome and uneconomical. The solvent method generally entails health and fire hazards, due to the toxicity and flammability of the solvent, and often the solution is not stable so that the results obtained therewith are not consistently reproducible. The dispersion method is troublesome in that it is difficult to get uniform dispersions and a uniform application of the agent to the fiber.

15 Now according to our invention, new chemical compounds are provided which not only have the useful property of inhibiting gas-fume fading of dyed cellulose acetate, but have the further admirable quality of being water-soluble in substance, but becoming converted into a water-insoluble form on the fiber. Our novel agents therefore are applicable from an aqueous solution, but are wash fast, and may be applied to the fabric either before dyeing, after dyeing or 20 as an adjuvant directly into the dye bath. In addition, our new compounds seem to have little or no effect on the light fastness of direct dyes, and therefore may be applied also to union fabrics containing, beside cellulose acetate, cotton or viscose fiber.

25 The novel compounds of this invention may be expressed by the general formula



40 wherein R stands for hydrogen or methyl, R' stands for hydrogen or methyl, n is an integer not greater than 2, while M designates a cation which will not impart water-insolubility to the compound; more particularly, M may designate the ammonium radical, an alkali-metal, magnesium, calcium or zinc.

45 They are generally produced by reacting the formaldehyde bisulfite of the corresponding cation with the corresponding diaryl-alkylene-diamine in aqueous alcoholic medium, and recovering the precipitated reaction product, although variations of this procedure are also applicable.

50 The products form readily solid hydrates and dissolve readily in cold water; but when the aqueous solution thereof is heated, they are de-

composed slowly to yield water-insoluble products, wherein the central alkylene radical and the two adjacent N-atoms are probably involved in an imidazolidine or a hexahydro-1,3-diazine ring. This conversion may be illustrated by the following typical equation:



Since dyeing of cellulose ester fiber is often accompanied by a steaming operation or is preceded by a boil-off operation, the opportunity for ring-closing the inhibitor is present, without introducing any special operations, if our novel compounds are applied to the fiber before dyeing or during the dyeing operation. If it is applied after dyeing, it may be developed by a simple steaming operation.

Without limiting our invention the following examples are given to illustrate our preferred mode of operation. Parts mentioned are by weight.

*Example 1.—Disodium salt of di-(N-methane sulfonate) of N,N'-diphenyl-ethylenediamine*

218 parts of sodium bisulfite were dissolved in 312 parts of water, 172 parts of 37% formaldehyde were added, and the resulting solution was held at 60° C.-65° C. for 30 minutes. The warm solution was then added to a solution of 212 parts of N,N'-diphenyl-ethylenediamine in 450 parts of 95% ethyl alcohol, and the charge was agitated at 65° to 70° C. for 4 hours. The reaction mass was allowed to cool to room temperature while agitating, and then the product was filtered off and washed with about 160 parts of alcohol. The cake was slurried with about 400 parts of benzene, then filtered off and dried. It consisted of a white solid, soluble in water. It had no definite melting point but charred when heated to a high temperature. Analysis showed it to be a tetrahydrate and to contain 1 atom of sulfur for each N-atom. Its structure, accordingly, corresponds most probably to the following formula:



This product may be used for the purpose of this invention, directly or after dehydration. In water, the compound decomposes gradually to yield 1,3-diphenyl-imidazolidine (see equation above), and but a small amount of the original diamine. Heat, acids and alkalis accelerate the decomposition. The mentioned imidazolidine may also be prepared directly from N,N'-diphenyl-ethylene diamine (Berichte, 31, 3255), and may be applied directly to cellulose ester fiber from an aqueous dispersion to produce an acid-fume fading stability of the same order as produced by N,N'-diphenyl-ethylenediamine itself.

*Example 2.—Di-potassium salt of di-(N-methane sulfonate) N,N'-diphenyl-ethylenediamine*

56 parts of potassium pyrosulfite were dissolved in 78 parts of water, and 42 parts of 37% form-

aldehyde were added. This solution was then added to 53 parts of N,N'-diphenyl-ethylenediamine dissolved in 112 parts of 95% ethyl alcohol. This mixture was agitated and heated at 65° to 70° C. for 3 hours. The charge after cooling was filtered. The filter cake was slurried with 160 parts of benzene on a steam bath, filtered hot, and dried. The product was a white powder, soluble in water. It had no definite melting point but charred at a high temperature. The product forms solid hydrates; in anhydrous form it is represented by the probable formula:



The product is similar in properties to that of Example 1, and may be used in the same manner and for the same purpose as the product of Example 1.

*Example 3.—Magnesium salt of di-(N-methane sulfonate) of N,N'-diphenyl-ethylenediamine*

22 parts of magnesium oxide were suspended in 156 parts of water, and sulfur dioxide was passed into the suspension until 70 parts had been adsorbed, the magnesium oxide going into solution. 81 parts of 37% formaldehyde solution were then added. This solution was added to a solution of 106 parts of N,N'-diphenyl-ethylenediamine in 225 parts of 95% ethyl alcohol. This mixture was agitated and heated at 65° to 70° C. for 3 hours. After cooling, the product was filtered off. The product was slurried with hot benzene and filtered. Analysis showed the product to contain 1 atom of sulfur for each atom of nitrogen. It is soluble in water, and its structure, in dehydrated state, probably corresponds to the formula—



It forms solid, water-soluble hydrates, and may be used for protecting dyed cellulose acetate against fume fading, in the same manner as the products of Examples 1 and 2.

*Example 4.—Disodium salt of di-(N-methane sulfonate) of N,N'-di-(m-tolyl)-ethylenediamine*

55 parts of sodium bisulfite were dissolved in 73 parts of water; 41 parts of 37% formaldehyde were added, and the mass was held at 60° C. to 65° C. for 30 minutes. This solution was added to a solution of 60 parts of N,N'-di-m-tolyl ethylenediamine in 130 parts of 95% ethyl alcohol. The mixture was agitated and heated at 65° C. to 70° C. for 3 hours. After cooling, the product was filtered off, slurried with hot benzene, filtered and dried.

The above product can be used in the dyeing procedure for cellulose acetate, giving good protection against fading by gas fumes. During the hydrolysis in the dyebath, the major portion is converted to 1,3-di-(m-tolyl)-imidazolidine, while a minor portion regenerates N,N'-di-(m-tolyl)-ethylenediamine.

*Example 5.—Disodium salt of di-(N-methane sulfonate) of N,N'-di-p-tolyl ethylenediamine*

12 parts of sodium bisulfite were dissolved in 16 parts of water, 8 parts of 37% formaldehyde were added, and the mass was held at 60° C. to 65° C. for 30 minutes. The solution was then added to 12 parts of N,N'-di-p-tolyl ethylenediamine dissolved in 48 parts of 95% alcohol. The

mixture was agitated and heated at 65° C. to 70° C. for 3 hours. After it had cooled to room temperature, the product was filtered off. The cake was slurried with warm benzene and filtered and dried. The product was soluble in water and was similar in properties to the meta isomer of Example 4.

*Example 6.—Di-sodium salt of di(N-methane sulfonate) diphenyl trimethylenediamine*

A solution of formaldehyde-sodium bisulfite (prepared by dissolving 23 parts of sodium bisulfite in 35 parts of water, adding 19 parts of 35.2% formaldehyde and heating at 60° C. for 30 minutes) was added to a solution of 21.2 parts of N,N'-diphenyl trimethylenediamine in 200 parts of 95% ethyl alcohol. This mixture was agitated and heated at 65° C. for about 2 hours. After cooling to room temperature, the product was filtered off and the cake washed with alcohol. The cake was then slurried with 120 parts of hot benzene, filtered and dried. Analysis showed the product to contain 1 atom of sulfur for each atom of nitrogen. It was soluble in water and was similar in properties to the product of Example 1, including the power to protect dyes on cellulose acetate against fume-fading.

*Example 7.—Di-sodium salt of di(N-methane sulfonate) of N,N'-diphenyl-1,2-propylenediamine*

A solution of formaldehyde-sodium bisulfite (prepared by dissolving 43 parts of sodium bisulfite in 62 parts of water and adding 32.4 parts of 35.1% formaldehyde) was added to a solution of 45.2 parts of N,N'-diphenyl-1,2-propyl diamine in 72 parts of ethyl alcohol. This mixture was agitated and heated at 65° C. to 70° C. for 4 hours. After cooling to room temperature, the solid material was filtered off and washed with alcohol. It was slurried with hot benzene and filtered. The product was a white solid, soluble in water. It is comparable as an anti-fume agent to the product in Example 1.

In a similar manner the omega sulfonates of N,N'-diphenyl-1,3-diamino butane, of N,N'-ditolyl-alkylene diamines, and of various other N,N'-diaryl-alkylene diamines may be readily prepared. Of chief interest in our present invention are those compounds which are capable of hydrolytic decomposition under the influence of heat, acids or alkalis to produce water-insoluble decomposition products. Those that have the general formula hereinabove set forth are especially valuable, because their hydrolytic decomposition produces chiefly a heterocyclic ring product, that is an imidazolidine or a hexahydro-1,3-diazine, which are characterized by good stability and water-insolubility. Addition of formaldehyde to the aqueous treatment bath aids in directing the hydrolytic decomposition toward production chiefly of said heterocyclic ring products, and suppresses the formation of other water-insoluble by-products.

It will be understood that the details of procedure may be varied widely within the skill of those engaged in this art. Thus, in lieu of the sodium, potassium or magnesium formaldehyde bisulfites, any metal bisulfite or pyrosulfite may be used which gives a water-soluble N-methane sulfonate.

Other solvents than ethyl alcohol may be used in the preparation of the methane sulfonates; for instance, propyl or butyl; or the reaction may be run in water, using an emulsifying agent such as

an alcohol-ethylene-oxide condensation product, polyglyceryl ricinoleate, cetyl trimethylammonium bromide, etc.

The order of adding the reactants may be varied. For instance, the solution of the diamine may be added to the formaldehyde-bisulfite solution; the sulfite solutions may be added to the alcohol solution of the amine followed by the formaldehyde; or the formaldehyde may be added and then the bisulfite.

The reactants may be mixed cold and then heated or they may be mixed warm. The temperature at which the reaction is carried out may vary widely (e.g., 50° C. to 125° C.), but the time will be longer if lower temperatures are employed.

Other solvents besides benzene may be used to wash out unreacted material, such as acetone, carbon tetrachloride, etc.

As already mentioned, our novel compounds may be applied to cellulose acetate material either before dyeing, during dyeing or as an after-treatment. For developing the inhibitor on the fiber, any regular steaming or boiling-off operation of the fiber may be taken advantage of, or a special steaming operation may be inserted. Our novel inhibitors may also be entered into the printing paste, where a printing process is resorted to, or they may be added to cellulose acetate rayon filaments.

The quantity to be applied will depend on the sensitivity of the dye to gas fumes and on the strength of the dyeing, the heavier shades generally requiring a greater degree of protection. But usually this quantity will be between 0.5% and 3% based on the weight of the dry cellulose acetate. In such limited quantities, the effect on the light fastness of direct colors is negligible, and consequently our novel agents may be employed safely in the dyeing of combination fabrics such as acetate and viscose or acetate and cotton.

The following additional examples will illustrate the mode of application of our novel compounds, it being however understood that no limitation is intended thereby.

*Example 8.—Application during dyeing*

0.035 gram of the blue dyestuff described in Example IX of U. S. P. 2,050,704 was pasted up with a commercial dispersing agent (a long-chain alcohol sulfate), and diluted with water at 100° F. to a volume of 250 cc. 0.4 gram of the anti-fume agent (from Example 1 above), dissolved in 500 cc. of warm water (100° F.) was then added, and the mixture was further diluted to a volume of 1 liter. A 20 gram piece of wet, previously scoured cellulose acetate satin was then entered; and dyeing was effected in the usual manner at 180° to 190° F. for one hour. The cloth was then rinsed with warm water and dried.

A similar piece of fabric was dyed in a similar bath except that no anti-fume agent was added.

When tested for atmospheric fading by standard methods, the fabric treated with our novel agent rated a color-fastness classification of 3 to 4 (good to very good), while the other sample rated 0 to 1 (very poor to poor).

*Example 9.—Application prior to dyeing*

A heavy-weight, highly delustered, all-cellulose-acetate fabric known in the trade as "taffeta," in greige condition as it comes from the weaving operation, was impregnated by the process known as padding, with a solution in water containing per gallon, 75 to 100 grams of our novel anti-fume agent (Example 1) and 0.25 to 1 oz. of a

dispersing agent (same as in Example 8), with the temperature of this liquor adjusted to between 100° and 120° F. Following padding, the cloth was passed between rolls set to permit the cloth to retain between 80% and 100% of its dry weight of the liquor, and then it was permitted to stand in the form of loosely-wound rolls for two hours at room temperature. Substantive fixation was then effected on the jig in the usual boil-off or scouring operation prior to the dyeing operation, this step consisting of treatment for 50 to 60 minutes at 160° to 200° F. in a water liquor containing per liter 2 to 4 grams of "Duponol D paste" (the aforementioned dispersing agent), 1 to 2 grams of soap and 0.75 to 1.25 grams of trisodium phosphate. Following the usual rinsings in water, the cloth was next dyed by conventional methods.

An additional quantity of the inhibitor (0.5 to 1% by weight based on the dry weight of the cloth) may be added to the dye bath, if desired. 20

Fabrics processed with the inhibitor by this procedure exhibit good resistance to atmospheric fading when subjected to the A. A. T. C. C. test method.

*Example 10.—Application in a printing process*

Printing pastes of the following composition were prepared:

| Paste                                   | A     | B     |
|-----------------------------------------|-------|-------|
| 1,4-diamino-2-methoxyanthraquinone..... | Parts | Parts |
| Glycerine.....                          | 0.25  | 0.25  |
| Water.....                              | 5     | 5     |
| Textile Gum.....                        | 40    | 35    |
| Anti-Fume Agent (Example 1).....        | 55    | 55    |
|                                         | None  | 5     |

These printing pastes were applied to cellulose acetate rayon cloth by the usual roller printing process with an engraved metal roll. The cloth was then dried, steamed for one hour in the cottage steamer without excess pressure, rinsed in warm water and dried.

When subjected to the A. A. T. C. C. test for fastness to atmospheric fading, the cloth printed with the printing paste B exhibited outstandingly better resistance than the cloth printed with the printing paste A.

*Example 11.—Application in a continuous process*

Pad liquors of the following compositions were prepared:

|                                                            | A            | B            |
|------------------------------------------------------------|--------------|--------------|
| 4-amino-4'-nitroazobenzene                                 | Parts<br>2.5 | Parts<br>2.5 |
| 4-nitro-4'-(ethyl, hydroxymethylamino) azobenzene          | 5            | 5            |
| The blue dye of Example IX, U. S. P. 2,050,704             | 5            | 5            |
| Anti-Fume agent (Example 1)                                | None         | 40           |
| Duponol D paste (same dispersing agent as in<br>Example 8) | 1            | 1            |
| Water                                                      | 986.5        | 946.5        |
| Total                                                      | 1,000.0      | 1,000.0      |

The temperature of these liquors was adjusted to 180° F., and separate pieces of an all-cellulose-acetate rayon satin were saturated with them by the padding process and then passed between rolls with a pressure to permit the cloth to retain about 70% of its dry weight of these liquors. In a continuous sequence, each cloth was then passed through another liquor known as the booster bath and which contained—

|                             | A     | B     |
|-----------------------------|-------|-------|
|                             | Parts | Parts |
| Pad liquor from above       | 2     | 2     |
| Anti-Fume Agent (Example 1) |       |       |
| Water                       | 98    | 96    |
| Total                       | 100   | 100   |

the temperature of the booster liquor being adjusted to 212° F., (the boiling temperature of water). Under this condition, steam was formed above the surface of the booster liquor and this steam being confined within an enclosed area served to fix substantively, both dye and inhibitor. The time of passage through the booster liquor and confined steam area may be adjusted as expedient. In this experiment, it was one minute, and was followed by rinsing the cloth in warm water and then drying.

When subjected to the A. A. T. C. test for fastness to atmospheric fading, the cloth treated in the B liquors exhibited much better fastness than the cloth treated in the A liquors.

25 Numerous other ways for applying our novel products are available and will readily suggest themselves to those skilled in the art. Thus, formaldehyde may be added to the treatment bath in optional quantity, say up to 1 mole for each mole of inhibitor employed, to aid in the hydrolysis of the inhibitor into imidazoline type compounds. Other details of our examples may 30 likewise be varied without departing from the spirit of this invention.

We claim as our invention:

- ### 1. A compound of the general formula



wherein R designates a member of the group consisting of hydrogen and methyl, R' designates a member of the group consisting of hydrogen and methyl, M is a cation which does not render the compound insoluble in water, and n is an integer not greater than 2.

- not greater than 2.

50 2. The di(alkali-metal) salt of di-(N-methane sulfonate) of N,N'-diphenyl-ethylenediamine.

3. The di(alkali-metal) salt of di-(N-methane sulfonate) of N,N'-diphenyl-1,2-propylene diamine.

55 4. A process for improving the color fastness of dyed cellulose ester fiber against acid-fume fading, which comprises treating said fiber with an aqueous solution of a compound as defined in claim 1, and then exposing the fiber to heat, to  
60 insolubilize the compound on the fiber.

DONOVAN ERB KVALNES.  
CARLTON WEBSTER CROCO.

#### REFERENCES CITED

The following references are of record in the file of this patent:

UNITED STATES PATENTS

|    | Number    | Name   | Date          |
|----|-----------|--------|---------------|
| 70 | 2,388,816 | Bean   | Nov. 13, 1945 |
|    | 2,416,380 | Collie | Feb. 25, 1947 |

#### OTHER REFERENCES

OTHER REFERENCES

75 1933 (1922).